

# UNITED STATES PATENT OFFICE.

ARTHUR CHARLES AUDEN, OF WESTMINSTER, LONDON, ENGLAND.

## METHOD OF EXTRACTING POTASSIUM SALTS FROM POTASSIUM-BEARING MINERALS.

1,334,940.

Specification of Letters Patent.

Patented Mar. 23, 1920.

No Drawing.

Application filed November 28, 1919. Serial No. 341,240.

To all whom it may concern:

Be it known that I, ARTHUR CHARLES AUDEN, of London, England, a subject of the King of Great Britain, residing at 5 5 Victoria street, Westminister, London, England, have invented certain new and useful Improvements in Methods of Extracting Potassium Salts from Potassium-Bearing Minerals, of which the following is a specification.

It is well-known that potassium compounds may be extracted from orthoclase feldspar by means of disintegration and treatment with heat when mixed with salt. 15 In some previous processes particularly British Patents Nos. 16,730<sup>99</sup> and 21,697<sup>11</sup> (Rhodin) only that class of potassium bearing mineral known as orthoclase feldspar has been used, but by the process hereafter 20 indicated by me silicates of aluminum and potassium such as orthoclase feldspar, pegmatite, mica and micaceous schist, muscovite, china-stone as also some forms of zeolite particularly those found in a basalt matrix 25 and also silicates of iron and potassium such as glauconite may be used.

The first step in the process is to crush the feldspar or other mineral so that it will pass through a half inch to a quarter inch mesh 30 as it is more economical of power to thus divide this process of obtaining a finely divided product into the two operations of crushing and grinding (milling) thus relieving the mill of the burden of large pieces 35 of material. I then prepare a mixture containing crushed feldspar 100 parts, slaked lime 56 parts, common salt 40 parts. Or the mixture may contain pegmatite 100 parts, slaked lime 60 parts, and common salt 42 40 parts; or it may contain china stone 100 parts, slaked lime 52 parts and common salt 48 parts; or mica, micaceous schist, or muscovite 100 parts, slaked lime 56 parts, common salt 45 parts; or glauconite 100 parts, 45 slaked lime 50 parts, common salt 50 parts. It is also practicable by this process to recover postassium compounds from leucite and alunite rock, but as this is more economically accomplished as a by-product in the 50 recovery of alum salts from the said leucite or alunite rock it is not included in this specification.

The mixture is then ground in a tube mill or similar machine to a fine powder, *i. e.*,

so that not more than 20 per cent., will be 55 left on an 180x180 mesh, that which is left on the mesh being returned to the mill and re-ground.

The mixture passed through the mesh is then gradually run into a furnace of the 60 ordinary muffle or inclined retort type where it is subjected to a temperature of 900°—1,000° C. for usually about one and a quarter hours. The time the mixture is in the furnace varies according to the nature of the 65 charge, as it is essential that it is uniformly roasted throughout and that only a limited proportion of "dead lumps" are formed, and these of small dimensions. I find that the time of heating necessary to get rid of the 70 whole of the "dead lumps" is unduly long and commercially uneconomical. I therefore only continue the heating for about one and a quarter hours and sieve out such dead lumps as remain. Poking or stirring 75 while in the retort must not be resorted to as this almost invariably leads to discoloration of the products and they are consequently spoiled for the purposes of sale. The charge must not be overheated as this 80 produces clinker, and if the mixture forms clinker the extraction of potassium compounds becomes practically impossible and, further, the clinkered particles are so hard that great damage is caused to the grinding 85 surfaces of the mills to which I shall presently refer. Further, the effect of this retardation of heating is that much less skill is necessary than by previous processes as it is not necessary again to roast until the 90 mass falls to a powder. It is quite possible with care and skill to roast the charge in the furnace so that no "dead lumps" as above mentioned are formed but this involves the charge being too long a time in the furnace 95 to be economical in working costs, and also the capital costs of the extra number of furnaces required for a given output is considerably greater than that of the sieving apparatus next hereafter described. The 100 limitation of the period of roasting so that the "dead lumps" are not all reduced is a special distinguishing feature of my invention.

After withdrawal from the furnace the 105 roasted mixture is placed on the cooling table, or platform, or is passed through a revolving cylinder and is allowed to cool

down, being spread in a thin layer and gently raked when cool enough not to fire the rakes. It is essential that no iron or metal rakes are used, as the result of the 5 action of the heat upon such rakes is to dis-color the products, the rakes are therefore made of hard beech wood. No cooling must at any time be permitted in the furnace even if the furnace is being stopped, say for the 10 purpose of repairs, as such cooling produces a mass of "dead" lumps. It will be found that the mixture at this stage is largely disintegrated, but there are some "dead" lumps formed in its passage through 15 the furnace, and it is therefore sieved, and the accumulated residue (not exceeding 20% as before) is re-ground in a secoad tube mill to the same fineness as that of the previous grinding, this suspension or cutting 20 short of the roasting and the sieving out of the lumpy residue is commercially preferable, and, by my process of selection by sieving, re-roasting and re-grinding of the residue only, the necessary fineness is obtained 25 at a very much decreased expenditure of fuel and time and wear of the mills.

The discharge from the sieving gear is then mixed and conveyed to a lixiviating vat or vats where it is thoroughly mixed with 30 clean hot water, *i. e.* usually about 75° C, until a new mixture is formed of the consistency of thick cream, particular care being taken that the mixture is thoroughly mixed and agitated and that no part is allowed to 35 settle in the form of a lump or cake in the bottom of the vat.

The above is the process when the raw material consists of silicates of aluminum and potassium but where the raw material is sili- 40 cate of iron and potassium such as glauconite the procedure is as follows at this point.

The discharge from the sieving gear is mixed and conveyed into a vessel capable of withstanding heat and pressure, *e. g.*, an 45 autoclave, into which high pressure steam and hot water are added and the whole thoroughly mixed and agitated, preferably by means of the revolution of the autoclave between trunnions thus saving the glands and 50 stuffing-boxes necessary for stirrers and the like.

The pressure of the steam at the autoclave inlet-valve should not be less than such as will yield a temperature of 200° to 205° 55 cent. Superheating of the steam may be resorted to if the above-mentioned pressure is not available but it must be carefully noted that the heat derived from such superheating must not exceed the maximum 60 of 25% of the total amount of heat required, the balance of 75% being yielded by the steam itself. Dry heating on one hand or boiling on the other both tend to reduce the amount of potash recoverable, and the for- 65 mer has the additional disadvantage of

forming "gobs" or "oysters" *i. e.*, slimy lumps, which prevent the rapid emptying of the vessel and make it very difficult to keep clean.

From the lixiviating vat or autoclave the 70 creamy mixture is pumped to a filter press but in the case where the raw material is china stone or similar materials, it is permissible to employ a settling and decantation plant through which the slurry is passed 75 prior to its being pumped into the filter press in order to relieve the filter press from treating all the material, the said decantation process separating out a proportion of the material which is not worth treating for 80 the extraction of potassium compounds which material is passed direct to the kneading machines to be hereafter described. In all cases it is permissible to use a vacuum filter in place of the filter-press but usually 85 it will be found that the press is the more economical to operate, particularly as regards the power absorbed.

The mixture is then pressed to a certain degree of consistency and is again washed 90 in water, the filter-press being fitted with through-washing apparatus for this purpose, the said water being of a higher temperature than that used in the lixiviating vats. This increase of temperature is at 95 this stage possible by reason of the filter-press, being a closed vessel, the increased temperature does not involve the loss by steam and vapor such as would occur if the higher temperature water had been used in 100 the open lixiviating vats, and this process is continued until the pressed mixture shows contents of chlorin about equal to 0.25 of sodium chlorid (NaCl) substantially as described in British Patent No. 21,697 of 1911. 105

The filter-press is at this stage cut off and this point marks the difference of the treatment of the residuals, I will first follow out my process for dealing with the potassium compounds.

The liquor from the filter-press is piped to an evaporator where the solution is concentrated. Particular care must be taken not to unduly hasten the process of evaporation and the temperatures used must never be 115 extreme or comparatively very great, as if this is done the product tends to be dis-colored and though its K<sub>2</sub>O contents are only slightdy chemically affected, the sale of a discolored product is very difficult and produces adverse market conditions. In the case where the raw material is silicate of iron and potassium which frequently contains phosphoric acid (P<sub>2</sub>O<sub>5</sub>) it is advisable to use two evaporators or sets of evaporators entirely separate as units but working in series, in order to eliminate the said phosphoric acid as one evaporator, even of large capacity, could not accomplish the separation of both the potassium compound and 130

the phosphoric acid so effectively and economically as two smaller evaporators working in series as here described, the potassium compound being obtained as a chlorid 5 and the phosphoric acid as a phosphate. The material is finally packed in barrels or bags—preferably the former—and it is important that any store should be kept dry and free from any marked changes of tem- 10 perature.

Secondly I will now follow out the process of preparing cement from the pressed mixture. After the liquor containing the potassium compound has been removed there 15 remains a damp, pressed and nearly solid mixture, which I refer to as the press-cake. This press-cake which must not be either too hard or too dry when taken from the filter-press, is mixed in a kneading or simi- 20 lar machine with lime which is preferably unslaked, but it must be carefully noted that this unslaked lime must be well ground to practically the same mesh as that first specified (20% residue on 180x180 mesh) 25 and also that considerably less volume of unslaked lime is needed than if the same be previously slaked, this difference in volume amounting to 25% in the case of very "fat" limes but from 18% to 20% may be taken as 30 the general average, but the principal reason why I use unslaked lime is that (1) it slakes itself in the kneading machine and mixes with the slurry therein very intimately and very rapidly, thus saving much time as also 35 power and depreciation of the machine, at least half an hour's continuous extra working of the machine frequently not producing such an intimacy of mixture. (2) The press-cake contains still a large amount of 40 water and the self-slaking of the unslaked lime creates heat which drives off quite a considerable percentage of the water in the form of steam, thus saving fuel and time in the furnace during the second firing about 45 to be described.

With regard to the amount of lime to be added, there are several conditions to be considered, most of such being decided by the market for the various grades of white 50 cement which can be produced, but in deciding the amount of lime to be added it is necessary to remember that from 45% to 55% of this lime is required as a constituent of the finished product (white cement) and, 55 weighing the lime before slaking, this means adding from 40 to 70 parts of lime (CaO) to each 100 parts (by weight) of press-cake as a dry substance, according to the properties, *e. g.* hard or soft, desired in the finished 60 product, and also adjustment must be made according as to whether the British standard or other specification is being worked to. It must be remembered, however, that the more lime that can be added—within of course 65 practical limits—the less risk of clinkering

and the formation of "dead lumps" there is in the final firing and consequently less wear and tear and power required in the final grinding and more passes through the sieves which does not need re-grinding. 70

This adjusted mixture is then passed through the kneading machine before-mentioned and the mixing in the machine is continued until all the constituents of the mass are distributed quite evenly. 75

When the adjusted mixture has been thoroughly kneaded and mixed, a small percentage of alum, *i. e.* alum cake, sulfate of aluminum, soda alum, or similar material equal to about 2½% of the dry weight of the 80 adjusted mixture, is added and the kneading and the mixing is continued until a thorough impregnation of the mixture with the alum is obtained, although the mixture of alum at this stage is not absolutely necessary. 85

The mixture is now placed in another furnace similar to that already described where it is heated for about two to two and a half hours, this second heating is a process of peculiar delicacy, the heat being gradually 90 and increasingly supplied, that is to say, there must be first applied the lowest temperature sufficient to dry out the moisture from the mixture; and the heat, as the moisture departs, must be gradually but continuously increased to about 1100° C., at which temperature the mixture must be treated for at least one hour. I have found in practice that in frequent cases one and a half hours were necessary, but the exact period varies 95 according to the material treated and the constitution of the mixture. An essential matter at this stage of the process is that careful provision must be made for the safe and free escape of the steam generated, and 100 to attain this the charge in the furnace must be firmly but not too tightly packed. 105

If it is too tightly packed the operation of the furnace is retarded and irregular, and the resultant composition is impracticable 110 for commercial purposes and spoiled. If on the other hand the charge is too loosely packed, pockets occur, gas and steam are retained therein and the whole process is ruined by reason of the irregular treatment 115 of the material.

When properly roasted, the contents of the furnace are discharged on to a cooling bed or platform as before, and, while cooling, are most carefully raked again with 120 beech wood rakes. After cooling, the resultant mass is again sieved to the mesh required by market conditions, the residue on the sieve which cannot pass must be again ground to attain the necessary fineness, 125 which fineness is the same as that determined by the said market conditions. The product of this second branch of the process may at this stage of the process be said to have become white cement. This white cement at 130

this stage, is generally too sensitive and quick setting for market conditions and its usefulness as a commercial product may be impaired, it is therefore almost always necessary to prepare gypsum, finely divided so as to pass through the same mesh as that used after the final mill discharge, and add from one and a half to two per cent., and well mix the same with the cement.

10 This mixture may be thinly spread on a floor for about a week and its quality is greatly improved if at the end of that period it is mixed and turned again in order that the particles shall be thoroughly aerated.

15 The amount of gypsum to be used varies in accordance with the market conditions and the use for which the white cement is desired and the time of aeration varies in accordance with the amount of lime in the 20 composition. The product is then finished and ready for packing in the casks or bags for despatch.

It is vital to the process that utmost cleanliness be rigidly observed, as any dirt, dust, 25 oil, rust, or detritus either in the potassium compound or the cement is seriously detrimental and is likely to deprive the product of its commercial value.

I claim as my invention:—

30 1. In the manufacture of potassium salts from potassium-bearing minerals, the method of incomplete roasting of a mixture of such potassium-bearing mineral, lime and salt, and the subsequent sieving out and re-grinding of the coarser parts of such roasted mixture, and the re-treatment of the whole of the re-ground material, by re-roasting, re-sieving and re-grinding, substantially as described.

40 2. In the manufacture of potassium salts from potassium-bearing minerals, where such potassium-bearing mineral contains silicate of iron and potassium, the treatment of a mixture, after roasting and sieving as described in claim 1, of the said potassium-bearing mineral, lime and salt, with steam and hot water in a closed vessel, and the agitation of the contents of the said closed vessel, substantially as described.

50 3. In the manufacture of potassium salts from potassium-bearing minerals, the method which consists in roasting a mixture of such potassium-bearing mineral, lime and salt, subsequently sieving out the coarser parts of such roasted mixture, re-grinding such coarser parts, and then re-treating the whole of the re-ground material by re-roasting, re-sieving and re-grinding, substantially as described.

60 4. In the manufacture of potassium salts from minerals containing silicate of iron and potassium, the method which consists in roasting a mixture of such material, lime and salt, sieving out the coarser parts of the 65 roasted mixture, re-grinding said coarser

parts, and treating the whole with steam and hot water in a closed vessel, substantially as described.

5. In the manufacture of potassium salts from minerals containing silicate of iron and 70 potassium, the method which consists in roasting a mixture of such material, lime and salt to a gradually increasing temperature of about  $1100^{\circ}$  C., sieving out the coarser parts of the roasted mixture, re- 75 grinding said coarser parts, and treating the whole with steam and hot water in a closed vessel, substantially as described.

6. In the manufacture of potassium salts from potassium-bearing minerals, where 80 such potassium-bearing mineral contains silicate of iron and potassium, the treatment of a mixture after roasting and sieving as described in claim 1, of the said potassium-bearing mineral, lime and salt, with steam 85 and hot water under pressure in a closed vessel, and the agitation of the contents of the said closed vessel, substantially as described.

7. In the manufacture of potassium salts 90 from minerals containing silicate of iron and potassium, the method which consists in roasting a mixture of such material, lime and salt, sieving out the coarser parts of the roasted mixture, re-grinding said coarser 95 parts, and treating the whole with steam and hot water under pressure in a closed vessel, substantially as described.

8. The herein described method of manufacturing white cement, which consists in 100 (a) roasting a mixture of potassium-bearing minerals, lime and salt, (b) the subsequent sieving out and re-grinding of the coarser parts of such roasted mixture, (c) the re-treatment of the whole of the re-ground material by re-roasting, re-sieving and re-grinding, (d) next treating the said 105 roasted material, which has passed through the sieve, with water to wash out the potash, (e) separating the wash-water from the 110 solid matter to bring the latter into the form of press-cake, (f) mixing lime with this press-cake under stirring and kneading, and (g) then subjecting this last-named mixture to roasting in a furnace, the product after 115 discharge from this last-named furnace being white cement, substantially as described.

9. The herein described method of manufacturing white cement from potassium-bearing minerals where such potassium-bearing minerals contain silicate of iron and potassium, which consists in (a) roasting a mixture of such potassium-bearing minerals, lime and salt, (b) the subsequent sieving out and re-grinding of the coarser parts 120 of such roasted mixture, (c) the re-treatment of the whole of the re-ground material by re-roasting, re-sieving and re-grinding, (d) next treating the whole with steam and 125 hot water in a closed vessel under agitation 130

of the contents of said closed vessel to wash out the potash and reduce the silicate of iron, (e) separating the wash water from the solid matter to bring the latter into the 5 form of press-cake, (f) mixing lime with this press-cake under stirring and kneading, and (g) then subjecting this last-named mixture to roasting in a furnace, the product after discharge from this last-named 10 furnace being white cement, substantially as described.

10. The herein described method of manufacturing white cement from potassium-bearing minerals where such potassium-bearing minerals contain silicate of iron and potassium, which consists in (a) roasting a 15 mixture of such potassium-bearing minerals, lime and salt, (b) the subsequent sieving out

and re-grinding of the coarser parts of such roasted mixture, (c) the re-treatment of the 20 whole of the re-ground material by re-roasting, re-sieving and re-grinding, (d) next treating the whole with steam and hot water under pressure in a closed vessel under agitation of the contents of said closed vessel 25 to wash out the potash and reduce the silicate of iron, (e) separating the wash-water from the solid matter to bring the latter into the form of press-cake, (f) mixing lime with this press-cake under stirring and 30 kneading, and (g) then subjecting this last-named mixture to roasting in a furnace, the product after discharge from this last-named furnace being white cement, substantially as described.

ARTHUR CHARLES AUDEN.